

## UNITED STATES PATENT OFFICE

1,940,602

PROCESS FOR THE MANUFACTURE OF  
ARTIFICIAL SILKAdrianus Johannes Leonard Moritz, Enka, N. C.,  
assignor to American Enka Corporation, New  
York, N. Y., a corporation of DelawareNo Drawing. Application October 3, 1932  
Serial No. 836,095

5 Claims. (Cl. 18—54)

My invention relates to the manufacture of a new type of colored artificial filaments more closely resembling those of natural raw silk.

More especially my invention concerns a method for giving a natural silk like lustre and improved dyeing qualities to filaments produced by the viscose process.

The object of the present invention is to provide a process whereby coloring chemicals may be incorporated into a viscose solution prior to the spinning thereof and whereby the resulting viscose solution is subsequently treated with a de-lustering agent.

Former inventions concerned the production of a low lustre filament by the use of pigments exclusively, but the use of pigments alone results in a thread which is physically weakened due to the necessity of employing a much larger percentage of the pigments than is necessary in my process.

The filaments obtained by using the prior processes does not resemble real silk since they are totally dull and lifeless in appearance.

The procedure followed in my invention does not result in a lowering of the physical properties and the filaments resulting from my process have a sub-surface lustre and covering power closely resembling those possessed by natural silk filaments.

Other objects will become apparent from a study of the following specifications and claims.

It should be noted that while I am describing my invention with reference to the viscose process, I do not wish to be limited thereto, since my process may be used in connection with any of the so-called wet-spinning processes.

In the preparation of the viscose solution, for spinning, cellulose is treated with an alkali solution to form alkali cellulose, which is allowed to ripen or age. The alkali cellulose is then subjected to the action of carbon bisulphide, to form a xanthate. This treatment usually lasts from 2-3 hours. Too short a treatment results in an unaltered alkali cellulose which will not dissolve.

In my new process I mix with the alkali cellulose or xanthate solution a watery dispersion of titanium oxide. Due to subsequent mixings and filtrations the fine particles of titanium oxide are dispersed equally throughout the viscose solution.

It has proved absolutely unnecessary to use oils or other agents to obtain a satisfactory dispersion of the pigments throughout the viscose solution. In the neighborhood of from 0.05 to 0.4% of titanium dioxide (calculated on the cellulose content of the solution) may be used.

The ripening and other steps, subsequent to the addition of the titanium oxide, result in the inclusion of these particles about from 24 to 72 hours prior to the time the solution is to be spun. Instead of titanium dioxide, I may use thorium oxide, wolfram oxide, zirconium oxide, or tin oxide.

Just prior to the spinning of the solution in order to produce artificial yarn, a small quantity of pine oil, usually less than 1.5% calculated on the total weight of the viscose, is added. I may also add a small amount of lanolin.

The resulting filaments have dispersed throughout separately, the finely divided pigment and oil. As a result, a filament which is colored, due to the presence of the particles of pigment, and which has a silk-like lustre due to the presence of the pine oil, is produced.

By experimentation I have found that when titanium oxide is employed in amounts less than 0.5%, it does not, of itself, produce a dull lustre yarn. The presence of the titanium oxide acts only to make the filaments less transparent. It has no effect on the surface appearance of the filaments, and the surface lustre of ordinary "high lustre" yarn remains.

When filaments which contain only titanium oxide are dyed black, dark blue, etc., and are compared with similarly dyed ordinary "high lustre" filaments, the dulling effect is not apparent and the resulting filaments in no way resemble natural silk.

My invention, therefore, lies in the combination of the two chemicals in the resultant filaments, the subsequent action of the oil producing a filament with a sub-surface lustre closely resembling real natural silk.

As examples of the manner in which my new invention may be carried out, the following are given:

*Example I.*—A watery paste of titanium oxide amount to 0.02% of the viscose solution is made up, and incorporated, by mixing, into the solution when it is first formed. The particles are thoroughly dispersed throughout the solution during this mixing and the subsequent filtrations, etc. After a period of approximately 60 hours the solution is in condition to be spun. Then about 0.9% of pine oil is added, the solution thoroughly mixed, and spun into filaments, films, etc.

*Example II.*—The process set forth in Example I is followed, but together with the pine oil, about 0.1% of lanolin, calculated on the viscose solution, is added to the solution.

Having now set forth my invention as required

by the patent statutes, what I desire to claim is:

1. In the manufacture of colored filaments, films, yarns and the like possessing a silk like lustre from cellulosic solutions the combination of the steps of incorporating into the solution, at the time it is made, from 0.05 to 0.4% of a pigment, calculated on the cellulose content, and then prior to spinning, adding to and mixing with the solution, less than 1.5% of pine oil, calculated on the viscose solution.

2. In the manufacture of colored filaments, films, yarns and the like from viscose solutions and possessing a silk like lustre, the combination of the steps of incorporating into the solution, at the time it is made from 0.05 to 0.4% of titanium oxide, calculated on the cellulose content, and then prior to spinning, adding to and mixing with the solution, less than 1.5% of pine oil, calculated on the viscose solution.

3. In the manufacture of colored filaments, films, yarns and the like possessing a silk like lustre from viscose solutions, the combination of the steps of incorporating into the solution, at the time it is made, from 0.05% to 0.4% of thorium oxide calculated on the cellulose content,

and then prior to spinning, adding to and mixing within the solution, less than 1.5% of pine oil, calculated on the viscose solution.

4. In the manufacture of colored filaments, films, yarns and the like possessing a silk like lustre from viscose solutions, the combination of the steps of incorporating into the solution, at the time it is made from 0.05% to 0.4% of wolfram oxide calculated on the cellulose content, and then prior to spinning, adding to and mixing within the solution, less than 1.5% of pine oil, calculated on the viscose solution.

5. In the manufacture of colored filaments, films, yarns and the like possessing a silk like lustre from viscose solutions, the combination of the steps of incorporating into the solution, at the time it is made, 0.4% or less of titanium oxide, calculated on the cellulose content, and then prior to spinning, adding to and mixing within the solution less than 1.5% of pine oil, calculated on the viscose solution, and a small amount of lanolin.

ADRIANUS JOHANNES  
LEONARD MORITZ.

100

30

105

35

110

40

115

45

120

50

125

55

130

60

135

65

140

70

145

75

150